

## UNITED STATES PATENT OFFICE

2,655,476

## THICKENED LUBRICANTS

Everett C. Hughes, Shaker Heights, and Ernest C. Milberger, Maple Heights, Ohio, assignors to The Standard Oil Company, Cleveland, Ohio, a corporation of Ohio

No Drawing. Application October 26, 1951,  
Serial No. 253,448

17 Claims. (Cl. 252—28)

This invention relates to a water-resistant, thickened lubricant in which the thickening agent is an inorganic substance.

Mineral lubricating oils are the most commonly used lubricants. Although they are available in various viscosity grades, they all possess flow properties which do not adapt them for many lubricating needs where a lubricant must adhere to the parts to be lubricated. For this reason, many proposals have been made for thickening the oils so that they will adhere to the surfaces to be lubricated, such as a wheel bearing.

A wide variety of materials has been proposed for addition to lubricating oils for thickening them. One of the materials most commonly used is soap, and soap thickened oils comprise the general class known as greases.

There are two general types of greases, those made with a calcium base soap and those made with a sodium base soap. The so-called soda base greases have relatively good temperatures susceptibility properties, that is, they retain their thickened properties at reasonably elevated temperatures. However, they deteriorate readily in the presence of water, presumably because the soda base soap is very soluble in water and the solution of the soap in water emulsifies with the oil. Greases made with a calcium soap, on the other hand, have better resistance to water, presumably because the calcium soaps are water insoluble. Calcium soap base greases, however, lose their consistency or thin out at elevated temperatures, presumably because the calcium soap becomes soluble in the oil as the temperature increases.

Both types of soap-base greases break down at high temperatures, of the order of 300 to 400° F. This breakdown is accompanied by an irreversible change in the grease structure, so that upon cooling the grease is observed to have lost its grease-like characteristics.

It has also been proposed heretofore (see Patent No. 2,260,625) to prepare a thickened lubricant by combining oil with an aerogel of a material not compatible with the oil, such as silica. These aerogel-thickened lubricants are far su- 45

2  
perior to the soap-base greases in stability at high temperatures as the following table shows:

TABLE I

|    | Soap or other thickener | Appearance at 400° F. | Appearance after cooling                                   |
|----|-------------------------|-----------------------|------------------------------------------------------------|
| 10 | Aluminum                | Very gummy and soft.  | Hard and lumpy.                                            |
|    | Lithium                 | Liquid                | Do.                                                        |
|    | Calcium                 | do                    | Hard—separation of soap.                                   |
|    | Sodium                  | do                    | Solidifies hard mass.                                      |
|    | Do                      | do                    | Soupy.                                                     |
|    | Sodium-calcium          | do                    | Complete separation of oil+soap.                           |
| 15 | Silica aerogel          | Unchanged             | Unchanged except somewhat thinner.                         |
|    | Do                      | do                    | Unchanged, upon stirring, breaks down into a heavy liquid. |

However, after heating at high temperatures some aerogel greases tend to lose consistency upon stirring and, further, most aerogel greases are particularly susceptible to deterioration in the presence of water, i. e., have poor water resistance. This is undesirable because there are many field applications where a grease is agitated or worked while subject to a high temperature and it is important that the grease retain its consistency under these conditions and subsequent thereto.

As will be explained hereinafter, the aerogel may be wetted by either oil or water, but is preferentially wet by water, and in the presence of water the oil phase leaves the aerogel and the thickening properties are at once destroyed.

It has been suggested that the water resistance of aerogel greases can be improved by incorporation therein of hydrophobic cationic surface-active agents, such as the higher aliphatic amines, quaternary ammonium compounds, polyamines, cyclic nuclear or extranuclear amines and their derivatives. It has been found, however, that not all of these compounds are effective water stabilizers under all conditions of use, especially severe conditions, and in addition that they do not have an advantageous effect on high temperature stability, and may even reduce or even destroy the high temperature stability of aerogel greases.

3

Accordingly, it is an object of the present invention to provide an aerogel-thickened lubricant having improved stability against the deleterious action of water under extraordinary conditions of use.

It is a further object to provide an aerogel thickened lubricant having improved water-resistance and also improved stability at high temperature, the two properties in which such greases are noticeably deficient.

are noticeably deficient. It is also an object to provide an additive capable of improving the water-resistance of aerogel-thickened lubricants.

thickened lubricants. It is a further object to provide an additive which not only is capable of improving the water-resistance, but is also capable of improving the high temperature stability of aerogel thickened lubricants. In this invention, it has been

In accordance with this invention, it has been discovered that the water resistance of a lubricating oil thickened with a non-abrasive, inorganic thickening or gelling agent, and particularly finely-divided silica, a silica aerogel being illustrative, can be improved by including in the composition a surface active, oil-dispersible, water-insoluble amino imidazoline of the general structure:



Many of the compounds having the above general structure are also capable of improving the high temperature stability of lubricating oils thickened with inorganic thickening or gelling agents, such as silica aerogels.

In the above formula, R is an aliphatic, cyclic or mixed cyclic-aliphatic amino group having at least one basic nitrogen atom, and preferably having at least two basic nitrogen atoms which can be primary, secondary or tertiary, in any combination of the three. Where one or more of the nitrogens is primary, i. e.,  $-\text{NH}_2$ , they can be attached at any position in an aliphatic chain or on a cyclic ring. Where one or more of the nitrogens is secondary or tertiary, i. e.,  $-\text{NH}$  or



they can be substituted in a straight or branched aliphatic chain, or in a heterocyclic ring, which can itself bear alkyl, alkylene, hydroxyalkyl or hydroxyalkylene groups, desirably in the 1-position, as in the above imidazoline ring. Thus R can be a mono, di- or tri-ethylene amino group, or a 1-alkylene-imidazoline group, or a 1-alkylene amino imidazoline group.

$R'$  is an alkyl, hydroxyalkyl, alkylene or hydroxalkylene group. prepared by reaction of

These compounds are prepared by reaction of aliphatic acids and polyamines followed by cyclization, in the following way:



Amino imidazolines in which R has two basic nitrogen atoms and from 4 to about 20 carbon atoms, such as diethylene diamino and triethylene triamino, and the alkyl-substituted N-alkylene and N'-alkylene-amino imidazolines (wherein R is attached to the imidazoline nucleus of the general formula through the N-alkylene or

N-alkyleneamino group), are readily available and are preferred. The chain length for R is dependent upon the basic (polar) character of the group; the larger the number of carbon atoms, relative to the number of amino nitrogens, the more the group takes on the character of a hydrocarbon and loses its basic or amine character. An upper limit of about 5 carbon atoms per amino nitrogen is indicated by this requirement, with about a maximum of 30 carbon atoms for the R group.

$R'$ , which is derived from an acid, can have from 11 to 21 carbon atoms, such as undecyl, tridecyl, abietyl, pentadecyl, undecenyl, heptadecyl, ricinoleyl, and heptadecenyl.

15 ricinoleyl, and heptadecenyl. The thickened lubricant containing these imidazolines has excellent temperature susceptibility properties which are characteristic of the silica aerogel greases, and in addition is highly resistant to deterioration by water.

The presence of the amino imidazoline also does not markedly affect the consistency of the thickened lubricant, i. e., the amount of the inorganic gelling agent to impart a given consistency to the thickened lubricant is not materially modified. Furthermore the inclusion of the imidazoline will not effect a change in the consistency of the thickened lubricant upon storage. This is to be contrasted with other materials which impart a lower initial consistency or a lower consistency on standing.

Due to the inorganic nature of the gelling agent, the thickened lubricant has excellent storage stability. This is to be contrasted with the heat susceptibility and deterioration of fatty materials in soap.

The preparation is simple and readily adaptable to continuous operation as contrasted with the involved grease-making techniques which are often considered in the industry as an art.

40 often considered in ...  
The oil stock used in making the thickened lubricant may be widely varied as contrasted with present grease-making requirements in which the oil in many cases is critical to meet certain specifications.

45 specifications. In addition, the avoidance of the use of soap permits the manufacturer to be independent of the supply, which is important in periods in which fats and soaps are scarce and many times of pronounced non-uniformity.

50 of pronounced ion. The inorganic gelling agent to be used in making the thickened lubricant in accordance with this invention may be any inorganic material which forms a gel with a lubricating oil and which is so finely divided as to be non-abrasive. 55 The preferred materials are the aerogels, which may be formed from any material not incompatible with oil, such as silica, alumina, and other gel-forming metal oxides.

60 A series of silica aerogels which can be used as the inorganic gelling agent of the invention are manufactured by Monsanto and marketed under the trade name "Santocel."

under the trade name Santocel. Santocel C is prepared from a sodium silicate solution in the following way: The solution is neutralized with sulfuric acid and then allowed to stand until the mixture sets to form a hydrogel. The by-product sodium sulfate is washed out by the repeated washings with water. The continuous water phase in this hydrogel is then replaced by continued washing with alcohol until an alcogel is formed. In order to remove the liquid phase without a collapse of the gel structure, the alcogel is placed in an autoclave which is then heated above the critical tempera-

ture of the alcohol and the pressure is allowed to increase to a point above the critical pressure of the alcohol. The vent valve is then opened and the alcohol allowed to escape. Under these conditions, the silica gel structure remains practically undisturbed and the liquid phase of the gel is replaced with air. The material is then reduced in particle size by blowing it through a series of pipes containing sharp bends with jets of compressed air. Santocel C has a secondary agglomerate particle size of about 3 to 5 microns.

Santocel A is prepared as set forth for Santocel C up to the point of removal of the product from the autoclave. This material is run through a continuous heating chamber where it is heated for  $\frac{1}{2}$  hour to a temperature of about 1500° F. to eliminate the last traces of volatile material. It is then broken down in a reductionizer or micronizer to a particle size of about  $\frac{1}{16}$  inch in diameter. The solids content of the original hydrogel used in preparing Santocel C is approximately 25% higher than that of Santocel A.

AR is a modification of A, differing only in that the material is reductionized to about the same particle size as C, approximately 1 to 6 microns in diameter.

ARD is a modification of AR, differing only in that ARD is densified by extracting air under vacuum, and therefore has a smaller volume than AR.

AX is an A which has not been devolatilized.

CDv is a C which has been devolatilized as set forth for Santocel A. The Santocel is reductionized before being devolatilized.

CDvR differs slightly from CDv in that the CDvR has been devolatilized just after heating in the autoclave and then reductionized. It differs from CDv in that the latter is reductionized before being devolatilized.

The primary differences between the A and C series are as follows:

1. The C's are prepared from a sodium silicate solution containing 25% more silica than the A's. Therefore, in general the A's are lighter and composed of smaller particles than the C's.

2. The A's have undergone a devolatilization step in their preparation.

The following are the bulk densities of several of the preferred silica aerogels:

|     |                        |                |
|-----|------------------------|----------------|
| AR  | Density, grams per ml. | 50             |
| ARD |                        | 0.029          |
| C   |                        | 0.055 to 0.064 |

In general, AR and ARD show superior gelling ability and the A's in general are better than the C's. Silica aerogels which have been devolatilized generally have a higher gelling efficiency than the undevolatilized aerogels.

Other types of inorganic gelling agents which may be used include a Fumed Silica marketed by B. F. Goodrich Company. It is finely divided and appears very much like an aerogel. It is made by a combustion or vaporization process, as a source of white "carbon black" for the rubber industry. The particles are several microns in size and porous in nature.

Another material is "Linde Silica Flour" marketed by Linde Air Products Co. It is very similar in physical appearance to the silica aerogel. The particle size of the silica is purported to be 0.01 to 0.05 micron and to be manufactured by burning silicon tetrachloride and collecting the combustion product on cool plates analogous to the production of carbon black. The particles

are thought to be aggregates or clusters of particles rather than of sponge-like character.

Still another inorganic gelling agent known as "Ludox" silica from DuPont, which is known as a silica sol, and silica derivatives thereof. It has a particular size of the order of 0.01 to 0.03 micron.

In preparing thickened lubricants it is necessary to remove the water from the sol and replace it with an oil. This is possible by formulating the lubricant and removing the water by flash distillation or azeotropic distillation.

No attempt is made to enumerate all of the inorganic gelling agents which will be suitable, nor to present examples of all of them since the novel aspects of the invention reside in waterproofing the lubricant rather than the use of novel gelling agents, per se.

The lubricating oil to be used in the process may have any lubricating viscosity. It may be raw oil, acid refined, or solvent refined, as required for the particular lubricating need.

The nature of the base oil has been found to make little difference in the relative consistencies of the thickened lubricants and conventionally (acid) refined oils produce slightly thicker lubricants than solvent-refined oils. Excellent working stability is obtained regardless of the type of the base oil. An increase in the viscosity of the base oil, as might be expected, brings increased viscosity to the thickened lubricant, and minimizes bleeding. The change is relatively small and fairly linear. The viscosity of the oil does not affect the working stability of the lubricant.

The relative proportions of the inorganic gelling agent and the oil will vary somewhat depending upon the desired body in the thickened lubricant, the gelling ability of the inorganic gelling agent and the viscosity of the oil used. It has been noted, for instance, that with the Linde silica flour, the lubricants are somewhat harder, i. e., have a lower penetration than lubricants containing the same weight of "Santocel." Lubricants made with low viscosity oils require a somewhat larger amount of the inorganic gelling agent to give a lubricant of the same penetration. The thickened lubricant may vary in consistency from the consistency of a slightly thickened oil to a solid or semi-solid of grease-like consistency. In general, the amount of the inorganic gelling agent falls within the range of 5 to 20%, and in most cases would fall within the range of 7 to 12%.

The amount of the inorganic gelling agent, as might be expected, affects the consistency of the thickened lubricant in that an increase in its concentration brings a corresponding increase in consistency. The range is fairly linear and the amount of the gelling agent can be selected with relation to the consistency desired in view of the information in the following examples. While the difference is slight, the lubricants made with lower concentrations of gelling agent possess better working stability, while lubricants with larger amounts of gelling agent show slightly improved temperature susceptibility characteristics. The bleeding tendencies are decreased by increasing concentrations of the gelling agent.

In general, the properties of the thickened lubricants are remarkably independent of the composition variables and are not critical. The relative concentration of the gelling agent affects the most significant alteration, particularly

7 with regard to the final consistency of the product. This permits the manufacture of thickened lubricants having a wide variety of consistencies.

A wide variety of oil-dispersible water-insoluble amino imidazolines can be employed in accordance with the invention to improve the water-resistance and high temperature stability of aerogel-base greases.

The imidazoline need not be oil-soluble, but it should be oil-dispersible. It should have a minimum boiling point of about 150° C. when its primary purpose is to stabilize the grease at high temperatures, but the boiling point is not material when only the water-stabilizing properties of the imidazoline are to be utilized.

The imidazoline is incorporated in the aerogel-base grease in a concentration ranging from 0.25 to about 1% by weight of the aerogel-base grease gives satisfactory results. There is no reason to employ more imidazoline than is necessary to achieve the desired effect, but excessive amounts do not harm, and amounts up to 5% or even higher have been successfully employed.

In some instances, the composition containing the amino imidazoline stabilizer may not display a long life when used continuously at high temperatures. A breakdown in high temperature stability at high temperatures if it appears is due to a decomposition, through oxidation, of the amino imidazoline stabilizer of the invention. In such circumstances, it is desirable to include in the composition an antioxidant for the amino imidazoline stabilizer. Conventional amine antioxidants which are more readily oxidized than the amino imidazoline of the invention can be employed for this purpose. Tetramethyldiaminodiphenylmethane, available under the trade name "Calco MB," is a particularly desirable antioxidant for the amino imidazolines of the invention. Only small quantities are required, and ordinarily an amount ranging from 0.1 to about 1% by weight of the aerogel base grease is ample. There is no reason to employ more antioxidant than is necessary to produce the desired effect, but excessive amounts do no harm and amounts up to 5% can be used, if desired.

The composition is made simply by mixing the inorganic gelling agent, the oil, the amino imidazoline, and the antioxidant in any order or manner.

In one embodiment, the amino imidazoline and, desirably, the antioxidant, can be incorporated with the inorganic gelling agent either by mixing directly or, if desired, by dissolving them in a volatile hydrocarbon solvent, such as pentane, adding oil, mixing the solution with the inorganic gelling agent, and then evaporating the solvent.

Generally, the amino imidazoline and, optionally, antioxidant are dispersed in the oil and the inorganic gelling agent added thereto and

mixed therewith. Any simple mixing technique can be employed and, if desired, the mixture can be homogenized in a colloid mill, although this is not necessary.

The composition of the invention is not limited to the oil, gelling agent and amino imidazoline. Any of the materials conventionally added to lubricants and greases can be included. The expression "consisting essentially of" as used herein is intended to refer to the components which are essential to the composition, namely, the oil, the inorganic gelling agent and the amino imidazoline, and the expression does not exclude other components from the composition which do not render it unsuitable for lubrication, such materials being, for instance, the antioxidant, high polymers to modify viscosity or viscosity index, materials to impart tackiness, lubricating solids such as graphite, antioxidant additives, corrosion inhibitors of various types, sulfur, additives to render the lubricant suitable for use in gears, for cutting, grinding, etc.

The following examples illustrate preferred embodiments of the invention:

#### Examples 1 to 18

Several amino imidazolines of the invention in a 0.8% concentration were incorporated in a thickened lubricant formed from:

30 8.0% silica aerogel (Santocel ARD).

0.8% imidazoline<sup>1</sup>.

0.5% Parafloc<sup>4</sup>.

0.5% methane base (antioxidant)<sup>3</sup>.

1.0% Paratac<sup>2</sup>.

0.01% dye.

89.19% solvent-extracted bright stock (150 SSU at 210° F.).

<sup>1</sup> The water-resistant aerogel base grease formula in Table II is as stated, the imidazoline being 1-β-hydroxyethyl-2-heptadecenyl imidazoline.

<sup>2</sup> An isobutylene polymer sold by the Enjay Company Inc. and commonly used in compounding greases.

<sup>3</sup> Tetramethyldiaminodiphenylmethane.

<sup>4</sup> A Friedel-Crafts reaction product, useful as a pour point depressant and sold by the Enjay Company, Inc.

A rigorous test to determine water stability was carried out on samples of the thickened lubricants. In accordance with this test a 2 x 2 in. stainless steel plate was coated with a uniform layer of the thickened lubricant, following which the coated plate was immersed in a beaker filled with tap water and boiled for a period of 60 minutes. A grease made only from oil and silica aerogel, for example (referred to in the table which follows as aerogel base grease) broke down immediately upon contact with the boiling water.

The thickened lubricant which according to an empirical visual observation was essentially unchanged in appearance was rated "very good" or "good." If the grease separated (oil to surface, gel to bottom) it was rated "bad" or "no water stability." If some emulsification was noted, but the grease was not disintegrated, it was rated "fair."

TABLE II

| Example No.                             | Additive structure                                                                          | Additive oil solubility | Water stability         |
|-----------------------------------------|---------------------------------------------------------------------------------------------|-------------------------|-------------------------|
| Aerogel base greases of the prior art:  |                                                                                             |                         |                         |
| 1. Lime soap grease.                    | None.                                                                                       |                         | Melts. Some separation. |
| 2. Aerogel base grease.                 | do.                                                                                         |                         | None.                   |
| 3. Water resistant aerogel base grease. | Amine O: 1-β-hydroxethyl-2-heptadecenyl imidazoline.                                        | Soluble.                | Good.                   |
| 4. Armeen 10 D (Armour).                | Primary amine:<br>90% C <sub>10</sub><br>8% C <sub>8</sub><br>7% C <sub>12</sub>            | do.                     | Bad.                    |
| 5.                                      | Cetyl dimethyl amine:<br>C <sub>16</sub> H <sub>33</sub> N(CH <sub>3</sub> ) <sub>2</sub> . | do.                     | Do.                     |

TABLE II—Continued

| Example No.                                                                                       | Additive structure | Additive oil solubility | Water stability                                                         |
|---------------------------------------------------------------------------------------------------|--------------------|-------------------------|-------------------------------------------------------------------------|
| Imidazolines which are not effective additives:<br>6.                                             |                    | Soluble                 | Very poor. Emulsification with water—sep. of oil and Santocel.          |
| 7.                                                                                                |                    | do                      | Very poor. Emulsification and sep. of oil and Santocel.                 |
| 8.                                                                                                |                    | do                      | No water stability. Complete sep. of oil and Santocel.                  |
| 9.                                                                                                |                    | do                      | Do.                                                                     |
| 10.                                                                                               |                    | Not soluble             | Very poor. Emulsification in water—sep. of oil and Santocel.            |
| 11.                                                                                               |                    | Partially soluble       | Very poor. Emulsification with water—sep. of oil and Santocel.          |
| 12.                                                                                               |                    | Soluble                 | Do.                                                                     |
| Amino imidazolines which are effective water stabilizers in accordance with the invention:<br>13. |                    | do                      | Very good.                                                              |
| 14.                                                                                               |                    | do                      | Good. Surface whitens. Some sep. of oil and Santocel. Still greaselike. |
| 15.                                                                                               |                    | do                      | Very good.                                                              |
| 16.                                                                                               |                    | do                      | Do.                                                                     |

TABLE II—Continued

| Example No. | Additive structure | Additive oil solubility | Water stability                                                 |
|-------------|--------------------|-------------------------|-----------------------------------------------------------------|
| 17.         |                    | Slightly soluble        | Very good.                                                      |
| 18.         |                    | Soluble                 | Do.                                                             |
| 19.         |                    | do                      | Do.                                                             |
| 20.         |                    | do                      | Do.                                                             |
| 21.         |                    | do                      | Do.                                                             |
| 22.         |                    | do                      | Do.                                                             |
| 23.         |                    | Not soluble             | Fair. Some emulsification and sep. of Santocel. Still a grease. |
| 24.         |                    | Not very good           | Very good.                                                      |

1 Derived by reaction of tall oil fatty acids with the corresponding diamine, as set forth in the reaction in column 3.

A comparison of the results of the water stability test (Table II) for Example 10 with Example 13, and Example 11 with Example 17, shows the importance of the 1-amino group in making the imidazoline and effective water stabilizer. Imidazolines lacking an amino group are ineffective, while imidazolines bearing such a group are very effective stabilizers. Further, a comparison of Example 14 with Example 15, shows that two basic nitrogen are better than one.

The determination of high temperature stability was made by placing approximately 100 cc. of grease in a 150 ml. beaker. The beakers were heated to the test temperature (400° F.) by placing them in an aluminum block furnace. This furnace consisted of a solid block of aluminum heated by internal electrical heaters. Six holes, each large enough to accommodate a 150 cc. beaker, were drilled into the top of the block, together with a thermocouple, so that a measure of the temperature of the block could be obtained.

55 In this manner, six beakers could be heated simultaneously. The beakers containing the grease were placed in the aluminum furnace and held there until the equilibrium temperature of the grease was 400° F. The samples were stirred at five-minute intervals during heating. After this the grease was allowed to cool to room temperature overnight and then was stirred vigorously with a spatula. Micropenetration measurements were obtained on the grease before and after the test procedure, and the results are expressed in the table below as per cent increase in penetration.

70 The micropenetration technique employed required a very small sample of grease. The microcone employed was specially built, and its dimensions are compared in Table II with those of the standard ASTM cone, ASTM designation 217-48, described on page 143 of the November 1948 edition of D-2 Specifications for Petroleum Products. The cone and grease cup em-

13  
ployed in obtaining the following test results required a minimum sample size of 35 ml.

TABLE III  
MICROCONE DIMENSIONS

|                                      | ASTM   |       | Sohio  |       | 10 |
|--------------------------------------|--------|-------|--------|-------|----|
|                                      | Cone   | Cup   | Cone   | Cup   |    |
| Diameter, mm                         | 65     | 78    | 20     | 43    |    |
| Height, mm                           | 45     | 45    | 17     | 24.5  |    |
| Depth, mm                            |        |       |        |       |    |
| Surface, sq. mm                      | 65     |       | 24.5   |       |    |
| Volume, cc.                          | 7,070  | 4,778 | 620    | 1,470 |    |
| Cone diam./cup surface               | 290    |       | 35.6   |       |    |
| Cone height/cup depth                | 0.0136 |       | 0.0136 |       | 15 |
| Wt. of assembly, gms.                | 0.693  |       | 0.693  |       |    |
| Wt. of assembly/sq. mm. cone surface | 150    | 13    |        |       |    |
|                                      | 0.021  |       | 0.021  |       |    |

<sup>1</sup> Calculated.

The following results were obtained on the aerogel base greases of Examples 1 to 18:

TABLE IV

| Example No. | Block performances |     |     |     |     | Percent increase |       |       |       |
|-------------|--------------------|-----|-----|-----|-----|------------------|-------|-------|-------|
|             | Orig.              | 1   | 2   | 3   | 4   | 1                | 2     | 3     | 4     |
| 2           | 54                 | 68  | 87  | 95  | 110 | 27.4             | 64.2  | 90.6  | 110.9 |
|             | 52                 | 67  | 87  | 107 | 103 |                  |       |       |       |
| 3           | 58                 | 87  | 126 | 149 | 153 | 58.5             | 121.2 | 159.3 | 173.7 |
|             | 60                 | 100 | 135 | 157 | 170 |                  |       |       |       |
| 10          | 64                 | 87  | 94  | 123 | 145 | 23.4             | 55.5  | 96.0  | 118.8 |
|             | 64                 | 78  | 105 | 124 | 135 |                  |       |       |       |
| 11          | 57                 | 96  | 150 | 189 | 238 | 50.0             | 159.3 | 218.6 | 297.3 |
|             | 56                 | 93  | 143 | 171 | 211 |                  |       |       |       |
| 12          | 54                 | 122 | 100 | 179 | 182 | 114.5            | 190.0 | 214.5 | 227.3 |
|             | 56                 | 114 | 159 | 167 | 178 |                  |       |       |       |
| 13          | 65                 | 91  | 98  | 103 | 111 | 28.6             | 49.6  | 66.9  | 71.4  |
|             | 68                 | 80  | 101 | 119 | 117 |                  |       |       |       |
| 14          | 54                 | 68  | 75  | 86  | 101 | 28.1             | 43.5  | 75.9  | 96.3  |
|             | 54                 | 65  | 80  | 104 | 111 |                  |       |       |       |
| 15          | 64                 | 81  | 123 | 132 | 141 | 29.2             | 81.5  | 106.2 | 117.0 |
|             | 66                 | 87  | 113 | 136 | 141 |                  |       |       |       |
| 16          | 65                 | 80  | 97  | 140 | 161 | 17.6             | 63.4  | 113.7 | 119.8 |
|             | 66                 | 74  | 117 | 140 | 167 |                  |       |       |       |
| 17          | 111                | 134 | 167 | 167 | 194 | 22.5             | 44.1  | 55.9  | 73.9  |
|             | 111                | 138 | 153 | 179 | 192 |                  |       |       |       |
| 18          | 73                 | 128 | 163 | 189 | 212 | 61.6             | 110.6 | 153.0 | 179.5 |
|             | 78                 | 116 | 155 | 193 | 210 |                  |       |       |       |
| 19          | 86                 | 110 | 159 | 179 | 207 | 21.3             | 70.1  | 94.8  | 127.0 |
|             | 88                 | 101 | 137 | 160 | 188 |                  |       |       |       |
| 20          | 81                 | 94  | 121 | 125 | 149 | 18.9             | 52.2  | 58.5  | 81.8  |
|             | 78                 | 95  | 121 | 127 | 140 |                  |       |       |       |
| 21          | 66                 | 91  | 113 | 114 | 145 | 35.6             | 63.6  | 72.7  | 102.3 |
|             | 66                 | 88  | 103 | 114 | 122 |                  |       |       |       |
| 22          | 72                 | 94  | 126 | 129 | 145 | 29.7             | 68.3  | 80.6  | 107.6 |
|             | 73                 | 94  | 118 | 132 | 156 |                  |       |       |       |
| 23          | 67                 | 81  | 100 | 120 | 146 | 23.0             | 53.3  | 81.5  | 111.9 |
|             | 68                 | 85  | 107 | 125 | 142 |                  |       |       |       |
| 24          | 92                 | 158 | 197 | 216 | 236 | 55.6             | 101.6 | 122.4 | 142.2 |
|             | 95                 | 135 | 180 | 200 | 217 |                  |       |       |       |

The importance of an amino group in the 1-position as regards both high temperature and water stability is evident in Table IV. Example No. 10 has a hydrogen in the 1-position, and Example No. 13 is similar to No. 10 but has a triethylene triamino group in the 1-position, and is much superior to No. 10. A comparison of Example 13 with Nos. 15 and 16 shows the group in the 2-position should have more than 11 carbon atoms for best high temperature stability. Examples Nos. 11 and 17 are an additional comparable pair, showing the critical nature of the 1-amino group. It will be noted that Examples 13, 17, 20, 21 and 22 are all superior to the aerogel base grease in high temperature stability, while retaining excellent water stability.

Examples 25 to 37

The following imidazolines can be substituted 75

14  
for any of the imidazolines in the greases of the preceding examples with good results:



| Example No. | Additive structure                                                                |
|-------------|-----------------------------------------------------------------------------------|
| 37-----     |  |

In the examples, the high temperature stability of the aerogel greases is tested by heating the greases to 400° F. This is an extreme test, inasmuch as the highest temperature to which a grease is subjected under even extraordinary conditions of use is about 300° F., but it was adopted as a suitable test standard by which to measure the high temperature stability of the greases because a grease stable at 400° F. will definitely have the stability necessary to withstand heating to 300° F. It will be understood that for normal purposes an aerogel grease need not be stable at temperatures above about 300° F., and that many of the greases of the invention at least meet this requirement. Where the term "high temperature stability" is used, it will be understood to mean that the aerogel grease is stable at at least 300° F.

While the invention is not to be limited to any theory or explanation, it may be of assistance in understanding the effect of the imidazoline on the water-resistance of the grease to explain that the inorganic gelling agent is either oil-wettable or water-wettable, but is preferentially water-wettable and has a great compatibility with water. When a lubricant thickened with an aerogel, for example, is contacted with water, the water replaces the oil in the gel and then separates from the oil. In accordance with the invention, the imidazoline, due to its surface activity, becomes attached to the silica and protects it from being wet by the water.

The imidazoline nucleus, since it possesses cationic character, is attracted to the anionic silica particles, with the result that the hydrophobic alkyl group of the molecule projects outward. Since water molecules are thus prevented from contacting the silica, the stabilizing agent, although less polar than water, is not eluted. However, the coated silica particles are easily wetted by oil since the long chain alkyl groups are oleophilic. Any mode of compounding the thickened lubricant which permits the imidazoline to come into contact with the inorganic gelling agent so as to protect it in this way, may be employed.

This application is a continuation-in-part of our application Serial No. 240,452, filed August 4, 1951 which is a continuation-in-part of application Serial No. 119,752, filed October 5, 1949, now abandoned.

We claim:

We claim:

1. A water-resistant thickened lubricant of good temperature susceptibility properties consisting essentially of a mineral lubricating oil of lubricating viscosity as the major component, an inorganic water-sensitive gelling agent imparting a grease-like consistency to the oil upon addition thereto as a minor component, and an oil-soluble, water-insoluble, surface-active polyamino imidazoline being in an amount less than the

16

16



where R is a radical containing an amino group and R' is selected from the group consisting of alkyl, alkylene, hydroxyalkyl and hydroxyalkylene groups.

2. A water-resistant thickened lubricant of good temperature susceptibility properties in accordance with claim 1, wherein R is diethylene amino.

3. A water-resistant thickened lubricant of good temperature susceptibility properties in accordance with claim 1, wherein R is triethylene amino.

4. A water-resistant thickened lubricant of good temperature susceptibility properties in accordance with claim 1, wherein R is an alkylene imidazoline group.

imidazoline group.

5. A water-resistant thickened lubricant of good temperature-susceptibility properties in accordance with claim 4, wherein R is an ethylene imidazoline group.

6. A water-resistant thickened lubricant of good temperature susceptibility properties in accordance with claim 4, wherein R is a diethyl-eneamino imidazoline group.

eneamino imidazoline group.

7. A water-resistant thickened lubricant of good temperature susceptibility properties in accordance with claim 1, wherein R' is ricinoleyl.

8. A water-resistant thickened lubricant of susceptibility properties in accordance with claim 1, wherein R' is ricinoleyl.

8. A water-resistant thickened lubricant of good temperature susceptibility properties in accordance with claim 1, wherein R' is heptadecyl.
9. A water-resistant thickened lubricant of good temperature susceptibility properties in accordance with claim 1, wherein R' is heptadecyl.

9. A water-resistant thickened lubricant of good temperature susceptibility properties in accordance with claim 1, wherein R<sub>1</sub> is hepta-decanyl.

10. A water-resistant thickened lubricant of  
good temperature susceptibility properties in ac-  
cordance with claim 1, wherein R' is undecyl,  
15 for imparting a grease-like

11. A composition for imparting a grease-like consistency to a mineral lubricating oil of lubricity, and also imparting stability.

consistency to a mineral lubricating oil, imparting viscosity, and also imparting stability against deterioration by water, comprising an inorganic water-sensitive gelling agent and an oil-soluble, water-insoluble, surface active poly-50 amino imidazoline having the formula:



where R is a radical containing an amino group and R' is selected from the group consisting of alkyl, alkylene, hydroxyalkyl and hydroxyalkylene groups, said compound being in an amount less than the gelling agent and imparting stability against deterioration by water.

65 12. A water-resistant thickened lubricant of  
good temperature susceptibility properties in ac-  
cordance with claim 11, wherein the imidazoline  
is.



13. A water-resistant thickened lubricant of

17

good temperature susceptibility properties in accordance with claim 11, wherein the imidazoline is:



14. A water-resistant thickened lubricant of good temperature susceptibility properties in accordance with claim 11, wherein the imidazoline is:



15

15. A water-resistant thickened lubricant of good temperature susceptibility properties in accordance with claim 11, wherein the imidazoline is:



25

16. A water-resistant thickened lubricant of good temperature susceptibility properties in accordance with claim 11, wherein the imidazoline is:



35

References Cited in the file of this patent

UNITED STATES PATENTS

| Number    | Name   | Date          |
|-----------|--------|---------------|
| 2,531,440 | Jordan | Nov. 28, 1950 |
| 2,554,222 | Stross | May 22, 1951  |

18

17. A water-resistant thickened lubricant of good temperature susceptibility properties consisting essentially of a mineral lubricating oil of lubricating viscosity as the major component, an inorganic water-sensitive gelling agent imparting a grease-like consistency to the oil upon addition thereto as a minor component and an oil-soluble, water-insoluble surface-active polyamino imidazoline being in an amount less than the gelling agent and imparting stability against deterioration by water and having the formula



where R is a radical containing an amino group and having from 4 to about 20 carbon atoms and R' is selected from the group consisting of alkyl, alkylene, hydroxyalkyl and hydroxyalkylene groups having from about 11 to about 21 carbon atoms.

EVERETT C. HUGHES.  
ERNEST C. MILBERGER.